

## UNITED STATES PATENT OFFICE

GEORGE A. RICHTER, OF BERLIN, NEW HAMPSHIRE, ASSIGNOR TO BROWN COMPANY,  
OF BERLIN, NEW HAMPSHIRE; A CORPORATION OF MAINE

## PRODUCTION OF PULP OF HIGH ALPHA CELLULOSE CONTENT

Application filed March 25, 1930. Serial No. 438,905.

No Drawing.

This invention relates to the production from raw cellulosic material, such as wood, of pulps which have an alpha cellulose content much higher than that present in the usual chemical wood pulps, such as sulphite or kraft, which accordingly constitute higher grade raw material for papermaking and for conversion into cellulose derivatives than the usual chemical wood pulps.

10 The process of the present invention, which is especially applicable to raw cellulosic material such as wood, comprises three cooking steps, but the first two cooking steps are not designed to effect fiber liberation, but to condition the wood so that it may be easily converted into a pulp of the desired character by the last cooking step. The wood employed as a raw material is cut into chips of the usual size employed for chemical pulping processes before being subjected to processing in accordance with the present invention. The initial step of the present process consists in cooking the wood chips at elevated temperature and under pressure in water, under which conditions the water extracts from the wood a large proportion of the pentosans present therein. The wood chips are then cooked short of fiber liberation in a suitable bisulphite liquor which 20 reacts upon and dissolves principally the lignous groups present in the wood. The wood chips are then cooked to complete fiber liberation in an alkaline liquor at elevated temperature and under pressure. The resulting product is characterized by its high alpha cellulose content, its low pentosan content, and its easy bleachability to whiteness with little loss of alpha cellulose. It is further characterized by a so-called solution viscosity much lower than that possessed by the usual chemical wood pulps, such low solution viscosity rendering it more suitable for use in the preparation of cellulose derivatives which are to be used as solutions of low viscosity in the production of such products as artificial silk, films, and lacquers.

40 A process such as the foregoing is advantageous, in that it necessitates the use of a comparatively low amount of expensive chemical in the production of cellulose pulp

of high market value. Thus, the extraction of pentosans from the raw wood with water makes possible the use of a liquor of comparatively low alkalinity in the last cooking step to complete fiber liberation and yet produces a product of high alpha cellulose content. Again, the process is simple and the total time of processing beginning with the raw wood chips and ending with the liberated pulp is no longer than the time consumed in those processes where refined wood pulps are produced by first liberating the fiber by a chemical pulping process such as the sulphite or so-called kraft process, and then digesting the liberated fiber in alkaline liquors, especially when the raw pulp is such, e. g., kraft pulp, as to require an additional treatment with agents such as chlorine water prior to digestion in the alkaline refining liquor. The initial treatment of the wood with superheated water, as previously stated, acts upon pentosans, but little, if any, ligneous matter is removed thereby. The ligneous matter is, however, so modified by this treatment that subsequent cooking with bisulphite liquor does not readily produce fiber liberation. Accordingly, it is easy to maintain the wood chips in the form of chips throughout the cooking operation with the bisulphite liquor, even though sufficient ligneous matter is removed therefrom so that after the final cook in an alkaline liquor to complete fiber liberation, the resulting pulp is of high cellulose content and is whitened by a comparatively light bleaching treatment. Evidently only a portion of the ligneous matter present in the wood responds to solution by the action of the bisulphite liquor, whereupon the rest of the ligneous matter, which has been modified by the action of the bisulphite liquor, readily responds to solution by the action of the alkaline liquor.

50 While various examples of procedure falling within the purview of the present invention are possible, I shall give for purposes of illustration only one example, which has been found to yield an eminently satisfactory product. Wood chips, e. g., spruce, are cooked in a closed digester in water for two to three hours at temperatures of from 250° to 400°

95

100

F., a temperature of about 325° F. representing one at which the desired extraction of pentosans from the wood proceeds at a satisfactorily rapid rate. The aqueous extracting liquor is then drained from the chips and the chips may, if desired, be washed with fresh water, but washing need not necessarily be practised. The water-extracted chips are then cooked short of fiber liberation in a suitable bisulphide liquor, for instance in a sodium or calcium base bisulphite liquor containing 1% combined and 5% free SO<sub>2</sub>, such a liquor corresponding to the liquors customarily used in the production of sulphite pulp. When cooking is effected at, say, 250° F. for about from two to four hours in such a liquor, the chips remain as such throughout the cooking operation, and show very little evidence of pulping, even though they are somewhat softer than the raw wood. Other types of acid sulphite liquors may be employed, for instance a sulphurous acid solution of sodium sulphate or sodium acid sulphate, in which case the liquor may also contain about 5% free SO<sub>2</sub>. If desired, the bisulphite liquor may be one containing a high combined SO<sub>2</sub> content in the form of a soluble bisulphite, such as sodium bisulphite, in which case the combined SO<sub>2</sub> may advantageously be approximately equal to the free SO<sub>2</sub> content of the liquor. For example, a bisulphite liquor containing approximately 4% free and 4% combined SO<sub>2</sub> may be employed, in which case the cooking of the chips is preferably effected at about 300° F., in order to promote the desired rate of removal of ligneous matter from the chips. After the cooking operation, the bisulphite liquor is drained from the chips and the chips are preferably washed to remove residual acid liquor and organic matter, so that alkali of the final alkaline cooking liquor will not be consumed in the neutralization of acid or associated organic matter. The washed chips are then cooked in an alkaline liquor of the type used in the so-called soda and kraft processes, but the alkalinity of the liquor may be much lower than the alkalinity of the cooking liquors of those processes wherein the liquors must accomplish reaction upon and solution of much more organic matter from the raw wood than that to be removed from chips which have been previously cooked as herein described. For example, the washed chips may be cooked to complete fiber liberation in about two to three hours, at a temperature of from 300° to 350° F. in a liquor containing only about 1.5 pounds of alkali per cubic foot, calculated as Na<sub>2</sub>O. The alkali is preferably made up of both caustic soda and sodium sulphide, the latter alkali being present to the extent of about 40%, which corresponds to the sulphidity of a typical kraft liquor. An alkaline liquor of such a composition makes possible the

production of a product having optimum physical characteristics, including a tear resistance comparable to, or even higher than, that possessed by the usual kraft pulp.

If desired, the bisulphite cook may be performed on the raw wood, whereupon the wood so cooked may then be extracted with superheated water, but this sequence of steps is ordinarily less desirable than that hereinbefore described, even though it leads to the product desired, as the active chemical of the bisulphite liquor is consumed in reacting upon and dissolving pentosans which might otherwise be reacted upon and dissolved by water alone. In other words, the process of the present invention is preferably practised with the water alone serving to extract as much undesirable non-fibrous matter from the wood as possible, so that the valuable chemical used in the subsequent cooking operations may be utilized for reaction upon and solution of only those wood components which are insoluble in superheated water alone.

I claim:

1. A process which comprises cooking raw cellulosic material short of fiber liberation in superheated water and in an acid sulphite liquor, and then cooking to complete fiber liberation in an alkaline liquor.

2. A process which comprises cooking raw cellulosic material in superheated water, then cooking short of fiber liberation in an acid sulphite liquor, washing, and cooking to complete fiber liberation in an alkaline liquor.

3. A process which comprises cooking wood chips in water at about 250° to 400° F., then cooking short of fiber liberation in an acid sulphite liquor, and cooking to complete fiber liberation in an alkaline liquor of comparatively low alkalinity.

In testimony whereof I have affixed my signature.

GEORGE A. RICHTER.

110

115

120

125

130